

**COPPER COATED URANIUM ARTICLE**

Allen G. Gray, Rocky River, Ohio, assignor to the United States of America as represented by the United States Atomic Energy Commission

No Drawing. Application January 6, 1945  
Serial No. 571,673

6 Claims. (Cl. 29—194)

This invention relates to the application of protective coatings on metallic uranium. The products produced in practicing this invention are useful in a neutronic reactor of the type described in the copending application of Fermi et al., Serial Number 568,904, filed December 19, 1944, which became U. S. Patent Number 2,708,565 on May 17, 1955.

Metallic uranium is an easily oxidizable metal which is readily corroded by atmospheric oxygen and by aqueous solutions. In order to protect the metal from the injurious effects of such media, it is desirable to provide a coating of some material which is less easily acted upon.

Many common protective coating materials are unsuitable for coating uranium; lead forms a pyrophoric alloy with uranium and for this reason its use is objectionable; some metals, such as tin, permit diffusion of the uranium through coatings of these metals with consequent impairment of their protective value; other metals form with the uranium, very brittle alloys containing many cracks and crevices which reduce their effectiveness.

It is an object of the present invention to provide protective coatings for uranium which are not subject to the defects enumerated above. A further object is to provide a barrier coating for uranium over which it is possible to apply various protective coatings that normally would be unsuitable because of their behavior toward the base metal. A further object of the invention is to provide highly protective electrodeposited coatings on metallic uranium.

In accordance with the present invention metallic uranium is provided with a protective coating comprising copper. The copper may be applied directly to the metal or to an intermediate coating of some other suitable metal possessing the property of adhering firmly to uranium and to copper. Nickel may be used to advantage for this purpose.

The metallic uranium preferably is prepared for the application of the coating by an etchant treatment of the metal surface with an aqueous etching solution containing chloride ions, for example a hydrochloric acid solution or a molten hydrate of ferric chloride. Particularly satisfactory treatments of this type involve anodic pickling of the metal in aqueous trichloroacetic acid solution, or aqueous phosphoric acid solution containing about ½% of hydrochloric acid, to remove a ½ to one mil layer of the surface metal. Prior to the etchant treatment the metal may be cleaned by sand-blasting, pumice-scrubbing, treating with organic solvents to remove grease or oily impurities, or treating with a chemical solvent for the oxide film on the metal. Aqueous nitric acid solutions containing from 30% to 55% HNO<sub>3</sub> by weight are especially useful for this purpose. An additional short treatment with this reagent should be applied after the etchant treatment in order to remove the coating of oxide or oxychloride from the etched metal surfaces.

The metallic copper coating may be applied by electroplating from conventional copper electroplating baths, such as acid copper, cyanide copper or pyrophosphate copper plating baths. The copper coatings of the inven-

tion may vary from exceedingly thin coatings of the order of 0.000015 inch up to 0.001 inch or more. The thickness of the coating should be selected appropriately to suit the subsequent treatment of the metal. Thus the thinnest coatings are normally employed in combination with relatively heavy coatings of other coating metals, whereas the heavy coatings are employed alone or in combination with additional metal coatings of moderate thickness.

10 The copper protective coatings are especially advantageous in that they inhibit diffusion of metallic uranium into other metals separated from the uranium by the copper. Thus the copper is particularly valuable as a barrier for preventing diffusion of uranium into protective coatings of lead, zinc, tin, cadmium, aluminum, and their alloys, and other metals of relatively low resistance to uranium diffusion.

In my U. S. patent application Serial No. 572,093 entitled, "Nickel Coatings and Method of Applying," filed 20 January 9, 1945, I have described uranium products provided with nickel protective coatings. Although the copper coatings of the present invention are superior to nickel coatings with respect to the barrier effect which they have upon diffusion of uranium, they can be substantially improved from the standpoint of corrosion resistance by combination with nickel coatings. Highly satisfactory combinations are disclosed and claimed in my application aforesaid. Other useful combinations are described and claimed herein.

30 Nickel provides coatings which adhere more firmly to uranium than copper coatings and consequently coatings of maximum adherence may be obtained by applying a first coating of nickel and a second coating of copper over the nickel. In this case the nickel is employed for its adhesive ability rather than its corrosion resistance.

Corrosion resistance may be secured by means of copper alone or by means of corrosion-resistant coatings applied over the copper. For example, copper constitutes a suitable base for application of lead coatings, which 40 provide protection against a wide variety of corrosive agents. The copper, by barring diffusion of uranium into the lead coatings, eliminates the possibility of the formation of a pyrophoric lead-uranium alloy which might otherwise be produced. The uranium-copper-lead bond is 45 also more secure than the uranium-lead bond, and a uranium-nickel-copper-lead bond is even more satisfactory.

While the protective value of lead alone is considerable, electroplated lead coatings have a somewhat porous structure permitting diffusion of corrosive agents into the 50 plating and consequently provide a less effective protection than is obtained with an impervious coating. By the application of a coating of copper and tin or copper and nickel over the lead platings their porosity can be reduced and their corrosion resistance increased.

55 An especially important improvement can be secured by electroplating a thin coating of tin upon an electroplated copper coating and then heating the tin to a temperature above its melting point but below the melting point of copper to cause the tin to diffuse into the pores of the copper plating. Very thin tin coatings, commonly termed "flash" coatings, the thickness of which may be from 0.000015 inch to 0.00005 inch, are suitable. Tin impregnated copper coatings prepared in this manner have been found to possess corrosion resistance many 60 times greater than simple copper-tin coatings. This technique is applicable to simple copper platings upon uranium as well as complex coatings such as the series nickel-copper-lead-copper. In the latter case the fusion treatment should be conducted below the melting temperature of the lead plating.

The copper coatings of the present invention have been found to be of very substantial value for use in com-

bination with chromium as a protective coating for uranium. While chromium has been found to produce firmly adherent coatings on smooth metallic uranium surfaces, the throwing power of chromium electroplating solutions is very low; hence, irregularities such as cracks, crevices, pinholes and the like in the metallic uranium surfaces are coated relatively slowly and the metallic uranium in such surface irregularities may be appreciably acted upon by the electroplating solution before the electroplated chromium layer attains protective proportions. The copper not only adds to the value of the finished coatings because of its barrier action but also protects fissures in the uranium metal surface from the chromium electroplating bath during the early period of electroplating with chromium. In order to afford protection for uranium during the chromium electroplating, it is not necessary to provide a thick copper layer since a copper flash coating has been found effective for this purpose.

It is normally expeditious to employ copper alone for the application of copper platings, but it is possible to effect similar results by employing mixed electroplating baths which apply two metals simultaneously. Thus by means of a copper-zinc electroplating bath brass coatings may be applied and these coatings possess barrier properties similar to those possessed by pure copper coatings.

#### Example 1

A machined uranium rod about 8 inches long and  $1\frac{1}{3}$  inch in diameter is prepared for electroplating by dipping in trichlorethene to remove grease, sand-blasting lightly, dipping in aqueous 35%  $\text{HNO}_3$  by weight at  $30^\circ \text{C}$ . for 4 minutes, rinsing with cold water, etching by anodic treatment in aqueous 50% trichloracetic acid solution at between  $50^\circ \text{C}$ . and  $60^\circ \text{C}$ . for 10 minutes at 50 amperes per square foot current density, rinsing with cold water, dipping for 4 minutes in cold aqueous 35%  $\text{HNO}_3$  solution to clean the etched metal surface, then rinsing in cold water.

The cleaned etched metal rod is immediately electroplated in a copper pyrophosphate electroplating bath comprising 75 grams per liter of copper as pyrophosphate at a current density of 25 amperes per square foot at  $60^\circ \text{C}$ . with air agitation until a copper plating about 0.001 inch thick is formed (about 60 minutes).

The uranium, treated as described, has a firmly adherent, continuous coating of copper, which for many purposes provides an adequate degree of protection against corrosion.

Since the copper electroplating is not as impervious as desirable for certain purposes it is improved in this respect by electroplating it in an aqueous tin electroplating bath comprising 90 grams per liter of sodium stannate at a current density of 25 amperes per square foot until a tin plating about 0.0001 inch thick has formed (about 10 minutes), then rinsing, drying, and heating at  $300^\circ \text{C}$ . for about 3 hours in Silicone #200 (a stable liquid polysilicone) bath to cause the tin to diffuse into the pores of the copper plating.

#### Example 2

A uranium rod copper-plated as in Example 1 is given a 0.001 inch nickel plating in an aqueous nickel sulfate electroplating bath comprising 240 grams per liter of nickel sulfate heptahydrate, 45 grams per liter of nickel chloride hexahydrate, and 30 grams per liter of boric acid, at a current density of 25 amperes per square foot for about 50 minutes. The uranium is thus provided with a protective coating of improved corrosion resistance.

#### Example 3

An extruded uranium rod about 4 inches long and 1.1 inches in diameter is prepared for electroplating by

dipping in aqueous 36%  $\text{HCl}$  solution for 20 seconds, then in aqueous 50%  $\text{HNO}_3$  solution for 15 seconds and finally in aqueous 36%  $\text{HCl}$  solution for 2 seconds. It is rinsed in cold water and electroplated in a nickel sulfate electroplating bath of the same composition as described in Example 2 for 15 minutes at about 25 amperes per square foot and ambient temperature to provide a nickel plating about 0.0003 inch thick.

The coated rod is rinsed with water and electroplated in a pyrophosphate type copper electroplating bath of the composition recited in Example 1 at a current density of 25 amperes per square foot at  $60^\circ \text{C}$ . until a "flash" coating of copper about 0.00003 inch thick has formed.

The copper-plated rod is again rinsed and then electroplated in a lead sulfamate electroplating bath comprising about 250 grams per liter of lead sulfamate at  $25^\circ \text{C}$ . at a current density of 25 amperes per square foot until a lead plating about 0.02 inch thick has formed (about 5 hours and 40 minutes).

This coating adheres firmly to the uranium. The copper provides a firm bond between the lead and the nickel and acts as a highly efficient blocking layer or barrier to diffusion of uranium into the outer lead layer. The thick lead layer provides very good protection against many corrosive agents.

Still greater protection is secured by electroplating a tin coating about 0.00005 inch thick over the lead to reduce its porosity. The tin is applied in the manner described in Example 1. It is preferred to provide an intermediate "flash" layer of copper by electroplating the lead-covered rod in an aqueous copper cyanide electroplating bath (a "strike") comprising 15 grams of copper cyanide per liter at  $40^\circ \text{C}$ . and at 50 amperes per square foot current density for 5 minutes, and to apply the tin over this copper layer. As in the copper-tin coating system of Example 1 the tin serves to fill the pores of the copper and this effect is increased and the corrosion resistance of the coating improved by a fusion treatment at about  $250^\circ \text{C}$ . for about 3 hours.

A somewhat similar but less effective coating is secured substituting a nickel plating for the tin plating.

#### Example 4

The process of Example 2 is repeated but in place of the lead electroplating step a zinc electroplating step is substituted using an electroplating bath containing 360 grams per liter of zinc sulfate at ambient temperature and a current density of 25 amperes per square foot until a zinc layer about 0.003 inch thick is applied (about 2 hours). The copper serves the dual function of improving adherence of adjacent metal layers and barring diffusion of uranium.

#### Example 5

A uranium rod is copper-plated as described in Example 1 but for only about 30 minutes. Over the 0.0005 inch copper plating (after rinsing) a chromium plating is applied by electroplating the copper-plated rod in a chromic acid bath containing 400 grams per liter of chromic acid at  $50^\circ \text{C}$ . and 250 amperes per square foot current density until a chromium layer 0.0005 inch thick has formed (about 30 minutes). A bright, smooth, even, firmly adherent composite electroplating is thus formed having especially valuable properties as a protective and barrier coating.

The novel coating processes described in this application are claimed in applicant's copending divisional application, Serial Number 190,672, filed on October 17, 1950.

It will be understood that I intend to include variations and modifications of the invention and that the preceding examples are illustrations only and in no wise to

be construed as limitations upon the invention, the scope of which is defined in the appended claims, wherein:

I claim:

1. A metallic uranium article protectively coated with successive layers of copper and lead.
2. A metallic uranium article protectively coated with successive layers of nickel, copper, and lead.
3. A metallic uranium article protectively coated with successive layers of nickel, copper, lead, and tin.
4. A metallic uranium article protectively coated with successive layers of nickel, copper, lead, copper, and tin.
5. A metallic uranium article having an electroplated coating of copper beneath an electroplated coating of chromium.
6. A metallic uranium article having a coating of electroplated copper impregnated with fused tin.

References Cited in the file of this patent

UNITED STATES PATENTS

|           |                  |               |
|-----------|------------------|---------------|
| 673,126   | Martin           | Apr. 30, 1901 |
| 1,147,718 | Hall             | July 27, 1915 |
| 1,559,077 | Guillaume et al. | Oct. 27, 1925 |
| 1,387,426 | Merritt          | Aug. 9, 1921  |
| 1,975,818 | Work             | Oct. 9, 1934  |
| 2,162,789 | Raub             | June 20, 1939 |

FOREIGN PATENTS

|         |        |              |
|---------|--------|--------------|
| 861,390 | France | Feb. 7, 1941 |
|---------|--------|--------------|

OTHER REFERENCES

Trans. Electrochem. Soc., vol. 66 (1934), page 41.